# EUROPEAN PATENT SPECIFICATION

(11) **EP 0 044 551 B1**
(45) Date of publication and mention of the grant of the patent: **27.06.1984**
(21) Application number: 81105699.3
(22) Date of filing: 20.07.1981
(51) Int. Cl.: F21K 5/02

(54) **Method of making a pressurized electrically-activated high-voltage photoflash lamp**
Verfahren zur Herstellung einer elektrisch zündbaren Blitzlampe mit Überdruck und hoher Spannung
Procédé de fabrication d'une lampe-flash à surpression et à allumage électrique haute tension

(30) Priority: 21.07.1980 US 170504
(43) Date of publication of application: 27.01.1982
(73) Proprietor: GTE Products Corporation, Wilmington, DE 19801 (US)
(72) Inventor: Armstrong, Donald E., Williamsport, Pa. (US); Sindlinger, Ronald E., Muncy, Pa. (US)
(74) Representative: Lemke, Jörg-Michael, Dipl.-Ing.

## Description

The invention relates to pressurized electrically-activated high-voltage photoflash lamps and particularly to a method of making such lamps.

Electrically-activated photoflash lamps are generally classified into two varieties: Low-voltage and high-voltage. Low-voltage photoflash lamps typically include a glass envelope with a combustion-supporting gas (e.g., oxygen) and a quantity of filamentary, combustible material (e.g., shredded zirconium) therein. A pair of electrically conductive lead-in wires are usually sealed in one end of the envelope and extend therein. A filament is utilized and interconnects the extending ends of the wires. When the filament is heated by a firing current usually generated from a low-voltage source such as battery or charged capacitor (e.g., having a voltage of from about 1.5 to 15 volts), it ignites a primer material which then ignites the combustible material to produce a flash of light. Naturally, the oxygen gas aids in the above ignition. In high-voltage lamps, the use of a filament is usually excluded by the provision of a glass or ceramic bead in which are located the extending ends of the lamp's conductive lead-in wires. Primer material serves to bridge the portions of these ends which project through the bead. High-voltage lamps also include the aforedescribed filamentary material and combustion-supporting gas. Flashing is accomplished by a low energy firing pulse approaching a few thousand volts and usually provided by a piezoelectric element. In another type of high-voltage lamp, the primer is located within an indention in the bottom of the lamp and the conductive lead-in wires extend therein.

The teachings of the present invention are particularly concerned with methods of making high voltage lamps.

In all of the above varieties of lamps, the conductive lead-in wires which form part of the lamp's ignition structure are typically sealed within one end of the lamp's envelope using a press (or "pinch") sealing operation during which the glass comprising this end portion is heated and compressed by a pair of opposing, parallel-faced metallic press members which converge to engage the heated glass and effect said compression. At least one engagement per lamp is required and on some occasions, two or three are employed. Examples of such lamps are illustrated in U.S. Patents 3,290,906 (Schilling et al), 3,752,636 (Warninck), 3,884,615 (Sobieski), and 4,059,389 (Armstrong et al). While such a technique has proven to successfully provide a hermetic seal of the metallic lead-in wires, the requirement of using a press seal possesses several drawbacks, particularly with regard to lamps having relatively small internal volumes (e.g., less than 1.0 cubic centimeter). Firstly, there exists a strong tendancy for the two wires to "swim" within the molten glass during pressing, which in turn can result in the two becoming misaligned. Secondly, a press-sealed end adds appreciably to the overall length of the lamp's envelope, a highly undesirable feature serving to defeat today's miniaturization efforts. Thirdly, the necessity for using a press seal adds to the overall costs of producing the lamp in that such a technique understandably requires complex lamp manufacturing equipment, which itself is both costly to produce and operate.

Accordingly, it is the object of the invention to provide a method of making an electrically-activated high-voltage photoflash lamp without the need for a press sealing operation. To obtain this object, the invention starts from a method for making a pressurized, electrically-activated low-voltage photoflash lamp such as disclosed in DE-C-1 254 963 and comprising securedly retaining an elongated glass tubing member having first and second opposing open end portions, positioning a pair of electrical conductors within said first open end portion such that said conductors project a predetermined distance within said glass tubing member, heating said first open end portion of said glass tubing member to a predetermined temperature to cause said first end portion to soften to allow to form a seal with said conductors without covering said conductors, permitting said heated first end portion to cool, applying a quantity of primer material to said conductors through said second open end portion, positioning a predetermined quantity of filamentary combustible material within said glass tubing member through said second open end portion, sealing said second end portion of said glass tubing member to provide a hermetically sealed envelope, and introducing a combustion supporting gas at an established pressure within said glass tubing member. In this prior art method the seal referred to was a press seal so that it obviously was not adapted to provide a solution for the object of the invention. Further, in this prior art method the pair of conductors are physically connected by a glass bead in addition to being physically connected by the filament. In addition, this prior art method required a copper tubing to be inserted into the press seal to be able to introduce the combustion-supporting gas into the glass tubing member after positioning the filamentary combustible material within said glass tubing member and sealing said second end portion.

To attain the object of the invention, this prior art method is rather revised in accordance with the invention in that the conductors do not engage the internal surfaces of said tubing member, the portions of said conductors projecting within said first open end portion not being physically connected, said softened end portion is allowed to assume a first position about said projecting conductors, a pressurized fluid is introduced within said glass tubing member through said second open end portion when said first end portion is heated to cause the sides of said heated first end portion located about said conductors to assume a second, expanded position about said conductors while retaining said seal therewith, said heated first end portion is permitted to cool while in said second, expanded position, said primer material is applied to the terminations of said conductors, and said combustion supporting gas is introduced through said second end portion of said glass tubing member prior to sealing thereof.

In a preferred embodiment of the invention the elongated glass tubing member is securedly retained so that said first open end portion is located vertically below said second open end portion prior to said positioning of said conductors, said electrical conductors positioned below said first end portion to project upwardly within said glass tubing member prior to said heating of said first open end portion; and in particular the electrical conductor may project upwardly in a vertical direction during said heating of said first open end portion.

There are several methods available to heat the first open end of the glass tubing member, preferably pressurized burners are used which only direct heat onto the external glass surfaces of said first open end portion of said glass tubing member during said heating step. The predetermined temperature attained during that heating step is preferably within the range from about 600 degrees Celsius to about 1150 degrees Celsius.

The pressurized fluid may be an inert gas, preferably selected from the group consisting of argon and nitrogen, but air may be used also as the pressurized fluid.

Also in a preferred embodiment the glass tubing member is evacuated through said second open end portion after positioning of said combustible material therein; it being highly advantageous to introduce the quantity of combustion-supporting gas within said glass tubing member through said second open end portion subsequent to said evacuation of said member then and prior to said sealing of said second open end portion.

### Brief description of the drawings

Fig. 1 is a front elevational view, in section, of an electrically-activated photoflash lamp produced in accordance with the teachings of the instant invention; and
Figs. 2-5 illustrate the various steps in carrying out the invention.

### Best mode for carrying out the invention

For a better understanding of the present invention, together with other and further objects, advantages and capabilities thereof, reference is made to the following disclosure and appended claims in connection with the above-described drawings.

With particular reference to Fig. 1, there is shown an electrically-activated photoflash lamp 10 manufactured in accordance with the preferred embodiment of the invention. Lamp 10 includes an hermetically sealed, light-transmitting glass envelope 11 having first and second opposing sealed end portions 13 and 15 respectively. Suitable glass materials for envelope 11 include G-1 type soft glass having a mean coefficient of thermal expansion of about 85 to 95×10⁻⁷ cm/cm/°k between 20°C and 300°C, and the harder boro-silicate glass recognized commercially as Corning type 7073, having a mean coefficient of thermal expansion of about 53.5x 1 0-7 cm/cm/°k between 0°C and 300°C. Borosilicate glass of this type possesses a typical composition of about 63.4% Si0₂, 7.2% AI_{Z}0₃, 17.8% B₂0₃, 0.6% LiO, 3.9% Na₂0, 4.6% K₂0, 2.2% BaO, and 0.2% CI. Another soft glass material successfully used in the invention is sold by the assignee of the instant invention under the product designation SG10 and is a potash soda lead glass having a typical chemical composition, by weight, of about 61% silica dioxide, 21.5% lead oxide, 7.7% sodium oxide, 7.45% potassium oxide 2.1% alumina oxide, 0.15% arsenic trioxide and 0.1% calcium oxide. SG10 glass also has a thermal expansion rating of 93.1, an annealing point of about 432 degrees Gelsius, a softening point of about 626 degrees Celsius, and a dielectric constant of 6.7. It is thus understood that the invention is capable of being successfully accomplished utilizing both soft and hard type glasses.

Located within envelope 11 is a quantity of filamentary combustible material 17 for providing a high intensity flash of light upon ignition thereof, the preferred material being shredded zirconium or hafnium. A quantity of about 2 to 40 milligrams is used although it is of course understood that the quantity of material 17 varies with the internal volume of envelope 11. Utilization of from 8 to 18 milligrams is preferred in lamps having envelopes with internal volumes equal to or less than 1.00 cubic centimeters, the preferred size for the envelopes of the present invention.

Also within envelope 11 is a combustion-supporting gas, e.g., oxygen, established at a pressure within the range of about 5 to about 15 atmospheres. The oxygen gas understandably serves to promote burning of shredded material 17 upon lamp ignition. Lamp 10 further includes an ignition means 19 disposed within end 13 for igniting the shredded zirconium or hafnium upon application of a suitable pulse as may be provided by a power source associated with many of today's electric cameras. One example of such a source is a piezoelectric element which is capable of providing a high voltage, low energy pulse approaching 5,000 volts. This element is typically located within the camera and provides said pulse through the camera's circuitry to a corresponding socket in which the photoflash device (which includes several lamps 10) is inserted. Accordingly, it is understood that the photoflash lamp produced in accordance with the teachings of the instant invention is adapted for use with multilamp photoflash devices which depend on high voltage, low energy pulses to achieve sequential ignition of the lamps contained therein.

Ignition means 19 includes a pair of spaced-apart electrical conductors 21 and 23 which are hermetically sealed within end 13 of envelope 11 and project therefrom. Accordingly, the aforementioned high voltage pulse is applied across conductors 21 and 23 to in turn ignite means 19, which in turn almost instantaneously ignites combustible 17. Conductors 21 and 23 are metallic wires having a diameter of 0,41 mm and are each comprised of a nickel iron alloy sold under the tradename Niron. An additional material especially preferred when using the aforementioned soft glass materials for envelope 11 is another nickel-iron alloy referred to as 52 alloy, which possesses a mean coefficient of thermal expansion of about 1 01.0x 1 0-7 cm/cm/°k between 25°C and 300°C. Still another acceptable material for this type of glass is Dumet, a well known nickel-iron alloy covered with a thin film (coating) of copper. When using the harder glass materials for envelope 11, conductors 21 and 23 were preferably formed from a metal alloy of iron, nickel, and cobalt, said material known commercially as Rodar or Kovar. This alloy has a composition which is approximately 54% Fe, 29% Ni, 17% Co, <0.5% Mn, <0.2% Si, and _{<}0.06% C and a mean coefficient of thermal expansion of about 50x 1 0-7 cm/cm/°k between 25°C and 300°C.

Each wire conductor 21 and 23 is hermetically sealed within first end 13 in accordance with the unique teachings of the invention (to be described below) and includes an enlarged, rounded termination portion 25 (Figs. 2-4) upon which is located the remaining portion of ignition means 19, a quantity of primer material 27. As shown in Fig. 1, primer 27 is positioned on both terminations to thus substantially cover same and be in electrical contact therewith. The circuit path between the spaced-apart conductors is provided by the shredded zirconium or hafnium, which thus bridges these members. It is also within the teachings of the invention to cover only one termination 25 with primer and connect this material with the remaining, exposed wire conductor termination 25. Still further, the invention permits the use of non-enlarged termination portions which may be located flush with the lower interior surface of envelope 11 (at end 13) with a single, large mass of primer 27 bridging the two terminations. Other alternative embodiments are well within the scope of the present teachings. Approximately two milligrams of primer 27 is used in the embodiment shown in Fig. 1, a preferred material comprising about 99% zirconium powder and 1% cellulose nitrite on a dried basis. The rounded, enlarged terminations are formed by applying a flame to each of the several ends of wires 21 and 23 to cause the ends to melt back to the rounded configuration depicted. Primer 27 is added to terminations 25 in the manner defined below.

Ignition of lamp 10 is achieved by application of the aforedefined high voltage pulse across the externally projecting ends of conductors 21 and 23 to cause an electrical breakdown of primer 27, resulting in a deflagration thereof and ignition of material 17. The total light output of finished lamp 10 is about 2,500 to 3,500 lumen-seconds although it is of course understood that this level can be either increased or decreased significantly by varying the quantities of zirconium (or hafnium), the internal envelope pressures, etc.

Dimensionwise, lamp 10 has an envelope external length of about 17,78 mm an external diameter of about 7,62 mm, and a wall thickness of about 0,813 mm. This substantially reduced size over many known comparative lamps makes lamp 10 especially adaptable to today's miniaturization efforts regarding multilamp photoflash devices.

In Figs. 2-5, there are illustrated the preferred steps in the method of making lamp 10. In Fig. 2, a preformed lead wire structure 31 is illustrated as being positioned within a holder 33 located below a vertically oriented elongated piece of glass tubing 35 having opposing open ends 37 and 39. Tubing member 35 preferably has an external diameter of 7,62 mm, and an internal diameter of 5,99 mm. It is understood that tubing member 35 is to eventually comprise the envelope 11 illustrated in Fig. 1. Accordingly, member 35 is comprised of one of the aforementioned glass materials. Member 35 is securedly retained within a second holder 41.

As illustrated, open end 37 is vertically positioned below the upper open end 39 and the pair of projecting ends of wire structure 31 are aligned so as to project vertically upward within end 37 and therefore inside of tubing member 35 a predetermined distance. It is understood that these projecting ends eventually comprise metallic lead wires 21 and 23 of the finished lamp 10. Accordingly, said projecting wires are given the numerals 21 and 23 in Figs. 2-5. Subsequent to sealing these projecting components within end 37 (to be described below), structure 31 is released from holder 33.

Prior to the above procedure, it is preferred to cover selected portions of terminations 25 with a glass frit coating (not shown) approximately 0,038 to 0,051 mm thick. The preferred frit, consisting of a fine powder of glass blended with a binder of amyl acetate and nitrocellulose, is prepared in slurry form and terminations 25 dipped therein. Air drying is used to dry the wet slurry coating prior to orientation within tubing member 35. As described in U.S. patent 4,059,389, frit coatings have been found to successfully prevent preignition short circuits across the lamp's conductors through the combustible material. A second feature of this material is that utilization thereof results in a near doubling of the primer breakdown voltage required to ignite lamp 10. This in turn assures a more reliable finished photoflash unit and a substantial reduction in production shrinkage. It is of course understood that when primer 27 is added to the terminations 25 having a frit coating thereon, selected regions of coating are removed to assure an electrical connection between the metal conductors and corresponding primer.

When using the glass tubing member 35 having the described internal diameter and wall thickness, it is preferred that conductors 21 and 23 project about 3,05 mm within open end 37. Once the conductors 21 and 23 are positioned therein in the manner illustrated in Fig. 2, heat is applied to pre-selected external areas of the open end portion 37 of tubing glass member 35 so as to raise the temperature thereof sufficiently to cause this end to soften, that is, to assume a plastic state. While in this state, end portion 37 (to comprise the first sealed end 13 of lamp 10) assumes a beaded form about the projecting wires 21 and 23 such that the wires are surrounded in the manner depicted in Fig. 3. It is believed that this beading action is the result of surface tension forces acting upon the glass while in the described plastic state. The surprising result is a hermetic seal of end portion 37 with the conductors 21 and 23 sealed and secured therein. As shown in Fig. 3, this unique procedure provided the defined seal without glass material covering the terminations of the respective wire members 21 and 23. The terminations (25) are thus free of glass and capable of providing the subsequent electrical contact with the lamp's primer material 27 (to be applied later).

The defined application of heat to tubing member 35 is preferably accomplished by utilization of a pair of opposing gas-oxygen burners 45 located on opposing sides of the cylindrical tubing member, each burner preferably adjacent a respective one of the wire conductors. Use of gas-oxygen or similar pressurized burners is preferred over other forms of heating (e.g., resistance type) because the forces exerted by the impinging flames against the heated external surfaces of member 35 serve to accelerate the aforedescribed deforming and sealing operation. The preferred temperatures for heating open end portion 37 are within the range of between 600 degrees Celsius and 1150 degrees Celsius, depending on the glass material utilized. It is of course only essential to heat the glass of the tubing member's first end portion to a temperature sufficient to cause it to assume the defined plastic (or softened) state such that it will flow about conductors 21 and 23. The resulting configuration (Fig. 3) assumed by the heated glass of first end 37, though forming a sound, hermetic seal with conductors 21 and 23, was not deemed totally satisfactory for use in lamp 10 because of its relatively reduced volume (caused by the indentations or depressions within the heated glass sides). Accordingly, it was surprisingly determined that this end portion could be expanded (while in the heated state) without sacrificing the hermetic seal attained. This was achieved by introducing a pressurized fluid within tubing member 35 through the remaining, upper open end 39. The preferred fluid used was air, however, inert gases (e.g., nitrogen, argon) could also be successfully used. The fluid was passed through a suitable nozzle 51 (Fig. 4) which was located immediately adjacent (or even partially within) end 39. The surprising end result was an expanding or "ballooning" of the heated glass sides of end portion 37 to a rounded configuration in the manner depicted in Fig. 4.

With regard to the invention, by the term pressurized is meant the introduction of a fluid within the open-ended tubular member to increase the internal pressure of the member and cause the described expansion or "ballooning" of the member's heated end 37. This increased pressure within the tubing member would inherently be greater than atmospheric. Nozzle 51 contained, in one example, an orifice 0,813 mm in diameter and was connected to a 533 mm steel manifold having an internal diameter of 25,4 mm. The pressure within the manifold was established at 222 N.

After permitting the glass to cool to room temperature, the resulting shape was also surprisingly found to be stronger than ends formed using the aforedefined press-sealing techniques, as indicated by scratch and upshock tests normally used to test small glass structures such as photoflash lamps. The most significant gain, however, was in overall internal volume for lamp 10 compared to a similar length envelope having a press-seal. A typical press-sealed end accounted for about 22% of the total envelope length. Using a seal made possible by the teachings of the invention, a similar length and diameter envelope realized a volume increase over the press-sealed envelopes of about 15 per cent. By way of example, an envelope having an overall length of 17,8 mm, an external diameter of 7,62 mm, and a wall thickness of 0,813 mm, realized a gain in internal length of about 1,52 mm over a comparative sized (externally) press-sealed envelope. Accordingly, it is possible to reduce internal pressure without altering the envelope's exterior dimensions. Alternatively, it is possible to produce lamps having reduced external features while maintaining the desired similar internal volumes. Still another highly advantageous feature of the invention is that it can be readily performed on existing photoflash production equipment without substantial modification thereto, as clearly indicated by the relatively simple components (e.g., holders 33,41) required.

In Fig. 5, there is illustrated the final steps of manufacturing lamp 10 in accordance with the teachings of the invention. The terminations of wires 21 and 23 have been coated with primer 27 using a suitable applicator (not shown) introduced through end 39. Subsequent to drying of the primer, the necessary quantity of filamentary combustible 17 is added, through open end 39. Any dispenser known in the art can be employed to locate material 17 and further definition is not believed necessary. This also holds true for the means of depositing primer 27. It is understood from the above that primer 27 is applied while in a liquid state and subsequently dries while in position. This drying can be facilitated by the introduction of heated air through second end 39. Additionally, the shredded zirconium or hafnium material 17 is inserted within open end 39 in order to frictionally engage the internal side walls of tubing member 35 in the manner illustrated in Fig. 5. Glass tubing member 35 is then evacuated through open end 39, a quantity of the described combustion-supporting gas (oxygen) is introduced within the member 35 through end 39, and end 39 is thereafter sealed using a tipping-off technique. Such a technique is well known in the art of manufacturing photoflash lamps and further definition is not deemed necessary. It is known, of course, that such a technique requires a "necking down" of the tubing member in the region of end 39 prior to final closure, thus resulting in a discarding of that portion of glass material above the constricted region and corresponding reduction from the original length to the desired 17,78 mm length for final envelope 11.

In the above technique, the upwardly projecting wires 21 and 23 were positioned within open end 37 so as not to engage the internal surfaces of this end portion of the glass tubing member. This alignment (Fig. 2) was considered necessary in order to accomplish the unique hermetic sealing described. It was also observed during all of the above techniques that direct exposure of wires 21 and 23 to the flames emitted by the gas-oxygen burners 45 on occasion resulted in the formation of a loose oxide layer on the wires. Such a layer could defeat formation of a sound hermetic seal between the glass and metal components and eventually result in gas leakage in the finished product. This potential problem was readily overcome by directing the burner flames only onto the designated glass surfaces (Figs. 2, 3). Understandably, utilization of other varieties of heaters may also prevent such an occurrence. The use of the gas-oxygen burners 45 is preferred, however, for the reason cited.

There has thus been shown and described a new and unique process for forming a hermetic seal within an end of a glass envelope between the glass and the photoflash lamp's metallic lead wires secured within the end. The described technique eliminates the need for the aforementioned press seal and therefore provides the several advantageous features described above.

## Claims

1. Method of making a pressurized, electrically-activated high-voltage photoflash lamp, said method comprising:
securedly retaining an elongated glass tubing member (35) having first (37) and second (39) opposing open end portions,
positioning a pair of electrical conductors (21, 23) within said first open end portion (37) such that said conductors (21, 23) project a predetermined distance within said glass tubing member (35), without engaging the internal surfaces of said tubing member (35), the portions of said conductors projecting within said first open end portion (37) not being physically connected, heating said first open end portion (37) of said glass tubing member (35) to a predetermined temperature to cause said first end portion (37) to soften to allow it to assume a first position about said projecting conductors (21, 23), to form a seal with said conductors (21, 23) without covering said conductors (21, 23), introducing a pressurized fluid within said glass tubing member (35) through said second open end portion (39) when said first end portion (37) is heated to cause the sides of said heated first end portion (37) located about said conductors (21, 23) to assume a second, expanded position about said conductors (21, 23) while retaining said seal therewith,
permitting said heated first end portion (37) to cool while in said second, expanded position,
applying a quantity of primer material (27) to the terminations of said conductors (21, 23) through said second open end portion (39),
positioning a predetermined quantity of filamentary combustible material (17) within said glass tubing member (35) through said second open end portion (39),
introducing a combustion supporting gas through said second end portion (39) at an established pressure within said glass tubing member (35), and
sealing said second end portion (39) of said glass tubing member (35) to provide a hermetically sealed envelope.

2. The method according to Claim 1 wherein said elongated glass tubing member (35) is securedly retained so that said first open end portion (37) is located vertically below said second open end portion (39) prior to said positioning of said conductors (21, 23) said electrical conductors (21, 23) positioned below said first end portion (37) to project upwardly within said glass tubing member (35) prior to said heating of said first open end portion (37).

3. The method according to Claim 2 wherein said electrical conductors (21, 23) project upwardly in a vertical direction during said heating of said first open end portion (37).

4. The method according to Claim 1 wherein said heating of said first open end (37) of said glass tubing member (35) is accomplished using pressurized burners (45) which only direct heat onto the external glass surfaces of said first open end portion (37) of said glass tubing member (35) during said heating step.

5. The method according to Claim 1 wherein said predetermined temperature is within the range of from about 600 degrees Celsius to about 1150 degrees Celsius.

6. The method according to Claim 1 wherein said fluid is an inert gas.

7. The method according to Claim 6 wherein said inert gas is selected from the group consisting of argon and nitrogen.

8. The method according to Claim 1 wherein said fluid is air.

9. The method according to Claim 1 further including the step of evacuating said glass tubing member (35) through said second open end portion (39) after said positioning of said combustible material (17) therein.

10. The method according to Claim 9 further including the step of introducing a quantity of combustion-supporting gas within said glass tubing member (35) through said second open end portion (39) subsequent to said evacuation of said member (35) and prior to said sealing of said second open end portion (39).

## Revendications

1. Procédé de fabrication d'une lampe à éclair à usage photographique à surpression et à amorçage commandé par haute tension électrique, caractérisé en ce que:
- on saisit fermement un tube de verre (35) de forme allongée ayant des première (37) et seconde (39) extrémités ouvertes,
- on met en place deux entrées de courant (21, 23) par la dite première extrémité ouverte (37), de manière que les dites entrées (21, 23) fassent saillie sur une longueur prédéterminée à l'intérieur du dit tube de verre (35) sans être au contact avec la paroi interne du dit tube (35), les parties des dites entrées pénétrant par la dite première extrémité ouverte (37) n'étant pas physiquement en contact,
- on chauffe la dite première extrémité ouverte (37) du dit tube de verre (35) à une température déterminée de façon à faire fondre la dite première extrémité (37) pour prendre une première position par rapport aux dites entrées (21, 23) et pour constituer un scellement avec les dites entrées (21, 23) sans recouvrir ces dernières,
- on introduit un fluide sous pression à l'intérieur du dit tube de verre (35) par la dite seconde extrémité (39) lorsque la dite première extrémité (37) est chauffée pour obliger la paroi de la dite première extrémité chauffée (37) autour des dites entrées (21, 23) à prendre une seconde position étendue par rapport aux dites entrées (21, 23) tout en maintenant le scellement,
- on laisse refroidir la dite première extrémité chauffée (37) tout en appliquant, dans la dite seconde position étendue, une quantité de matériau d'amorçage (27) sur les extrémités des dites entrées (21, 23) par la dite seconde extrémité ouverte (39),
- on met en place une quantité déterminée de clinquants combustibles (17) à l'intérieur du dit tube de verre (35) par la dite seconde extrémité ouverte (39),
- on introduit par la dite seconde extrémité ouverte (39) un gaz favorisant la combustion sous une pression déterminée, et
- on scelle la dite seconde extrémité (39) du dit tube de verre (35), de manière à constituer une ampoule hermétiquement fermée.

2. Procédé selon la revendication 1 caractérisé en ce que l'on maintient fermement le dit tube de verre de forme allongée (35), de telle manière que la dite première extrémité ouverte (37) soit disposée verticalement sous la dite seconde extrémité ouverte (39) avant de mettre en place les dites entrées de courant (21, 23) qui sont disposées sous la dite première extrémité (37) pour faire saillie vers le haut à l'intérieur du dit tube de verre (35) avant de chauffer la dite première extrémité ouverte (37).

3. Procédé selon la revendication 2 caractérisé en ce que les dites entrées de courant (21, 23) font saillie verticalement vers le haut pendant le chauffage de la dite première extrémité ouverte (37).

4. Procédé selon la revendication 1 caractérisé en ce que l'on chauffe la dite première extrémité ouverte (37) du dit tube de verre (35) au moyen de chalumeaux (45) dirigeant la chaleur uniquement sur la paroi extérieure de verre de la dite première extrémité ouverte (37) du dit tube de verre (35) pendant l'étape de chauffage.

5. Procédé selon la revendication 1 caractérisé en ce que la dite température déterminée est comprise entre 600 et 11 50°C environ.

6. Procédé selon la revendication 1 caractérisé en ce que le dit fluide est un gas inerte.

7. Procédé selon la revendication 6 caractérisé en ce que le dit gaz inerte est aussi bien de l'argon que de l'azote.

8. Procédé selon la revendication 1 caractérisé en ce que le dit fluide est de l'air.

9. Procédé selon la revendication 1 caractérisé en ce qu'il inclut en outre une étape au cours de laquelle on fait le vide à l'intérieur du dit tube de verre (35) par la dite seconde extrémité ouverte (39) après avoir disposer les dits clinquants combustibles à l'intérieur.

10. Procédé selon la revendication 9 caractérisé en ce qu'il inclut en outre une étape au cours de laquelle on introduit une quantité de gaz favorisant la combustion par la dite seconde extrémité ouverte (39) après avoir fait le vide dans le dit tube (35) et avant de sceller la dite seconde extrémité ouverte (39).

## Patentansprüche

1. Verfahren zum Herstellen von unter Druck stehenden, elektrisch aktivierten Hochspannungs-Photoblitzlampen, bestehend aus:
sicherem Haltfern eines länglichen Glasröhrenelementes (35) mit einem ersten (37) und einem zweiten (39) offenen Endteil, die einander gegenüberliegen,
Positionieren von zwei elektrischen Leitern (21, 23) innerhalb des ersten offenen Endteils (37) in der Weise, daß die Leiter (21, 23) eine vorgegebene Distanz in das Glasröhrenelement (35) vorstehen, ohne an den Innenflächen des Röhrenelementes (35) anzuliegen, wobei die Teile der Leiter, die in den ersten offenen Endteil (37) vorstehen, körperlich nicht verbunden sind,
Erwärmen des ersten offenen Endteils (37) des Glasröhrenelementes (35) auf eine vorgegebene Temperatur, um zu bewirken, daß das erste Endteil (37) erweicht, so daß ihm möglich ist, eine erste Position um die vorstehenden Leiter (21, 23) anzunehmen, um eine Dichtung mit den Leitern (21, 23) zu bilden, ohne die Leiter abzudecken (21,23),
Einführen eines unter Druck stehenden Strömungsmittels in das Glasröhrenelement (35) durch den zweiten offenen Endteil (39) während der erste Endteil (37) erwärmt ist, um zu bewirken, daß die Seiten des erwärmten ersten Endteils (37), die um die Leiter (21, 23) herum angeordnet sind, eine zweite, expandierte Position um die Leiter (21, 23) annehmen, während die Abdichtung damit beibehalten wird,
dem erwärmten ersten Endteil (37) wird erlaubt, sich abzukühlen, während er in der zweiten, expandierten Position ist,
Anlegen einer Menge Zündermaterial (27) an die Enden der Leiter (21, 23) durch den zweiten offenen Endteil (39),
Positionieren einer vorgegebenen Menge eines fadenförmigen verbrennbaren Materials (17) in das Glasröhrenelement (35) durch den zweiten offenen Endteil (39),
Einführen eines verbrennungsfördernden Gases durch den zweiten Endteil (39) mit einem vorgegebenen Druck in das Glasröhrenelement (35), und
Abdichten des zweiten Endteils (39) des Glasröhrenelementes (35) um einen hermetisch dichten Kolben zu schaffen.

2. Verfahren nach Anspruch 1 bei dem das längliche Glasröhrenelement (35) fest derart gehaltert wird, daß das erste offene Endteil (37) vertikal unterhalb des zweiten offenen Endteils (39) lokalisiert ist, ehe die Leiter (21, 23) positioniert werden, wobei die elektrischen Leiter (21, 23) unterhalb des ersten Endteils (37) positioniert sind, um nach oben in das Glasröhrenelement (35) vorzustehen, ehe der erste offene Endteil (37) erwärmt wird.

3. Verfahren nach Anspruch 2 bei dem die elektrischen Leiter (21, 23) während der Erwärmung des ersten offenen Endteils (37) in vertikaler Richtung nach oben vorstehen.

4. Verfahren nach Anspruch 1 bei dem die Erwärmung des ersten offenen Endes (37) des Glasröhrenelementes (35) unter Verwendung von Druckbrennern (45) durchgeführt wird, die Wärme nur auf die äußeren Glasoberflächen des ersten offenen Endteils (37) dss Glasröhrenelementes (35) während des Erwärmungsschrittes richten.

5. Verfahren nach Anspruch 1 bei dem die vorgegebene Temperatur im Bereich von etwa 600° Celsius bis etwa 11 50° Celsius liegt.

6. Verfahren nach Anspruch 1 bei dem das Strömungsmittel ein inertes Gas ist.

7. Verfahren nach Anspruch 6 bei dem das inerte Gas aus der aus Argon und Stickstoff bestehenden Gruppe ausgewählt wird.

8. Verfahren nach Anspruch 1 bei dem das Strömungsmittel Luft ist.

9. Verfahren nach Anspruch 1, das weiter den Schritt aufweist, das Glasröhrenelement (35) nach dem Positionieren des verbrennbaren Materials (17) durch das zweite offene Endteil (39) zu evakuieren.

10. Verfahren nach Anspruch 9, das ferner den Schritt aufweist, eine Menge verbrennungsförderndes Gas im Anschluß an die Evakuierung des Elementes (35) und vor dem dichten Verschießen des zweiten offenen Endteils (39) eine Menge verbrennungsförderndes Gas durch das zweite offene Endteil (39) in das Glasröhrenelement (35) eingeführt wird.
